# EUROPEAN PATENT SPECIFICATION

(11) **EP 0 369 804 B1**
(45) Date of publication and mention of the grant of the patent: **18.09.1996**
(21) Application number: 89311907.3
(22) Date of filing: 17.11.1989
(51) Int. Cl.: C10M 141/10, C10M 163/00, C10N 30/06

(54) **Lubricant method and compositions**
Schmierverfahren und Zusammensetzung dafür
Méthode de lubrification et compositions pour l'effectuer

(30) Priority: 18.11.1988 GB 8826961
(43) Date of publication of application: 23.05.1990
(73) Proprietor: CASTROL LIMITED, Swindon Wiltshire SN3 1RE (GB)
(72) Inventor: Hutchings, Timothy, Wantage Oxfordshire OX12 0QG (GB); Green, David, Wallingford Oxfordshire OX10 0PD (GB); Carter, Brian Howell, Reading Berkshire RG8 7SR (GB)
(74) Representative: Eyles, Winifred Joyce

(56) References cited:
- EP-A- 0 239 088
- EP-A- 0 267 875
- GB-A- 749 678
- US-A- 3 254 027
- US-A- 3 899 432
- US-A- 4 137 187
- US-A- 4 431 552

## Description

This invention concerns the lubrication of crosshead diesel engines, for example marine slow speed crosshead diesel engines.

The lubrication of crosshead diesel engines, and in particular the cylinder liners and piston rings of such engines, presents problems since the temperatures and pressures involved during their operation can lead to breakdown of the film of lubricant on the internal walls of the cylinder liners. When this occurs it leads to excessive cylinder liner and/or piston ring wear.

Various additives have been proposed for lubricant compositions for engines for the purpose of reducing engine wear. Anti-wear additives, for example, have been proposed but although they are effective at low temperatures, they tend to become ineffective at the temperatures encountered at the top of the cylinder liners of crosshead diesel engines.

Extreme pressure additives have also been proposed which function as the lubricant film breaks down between metal surfaces when they slide under high pressures. They are in particular proposed for use in gear oils. The disadvantages of using such additives in lubricant compositions for crosshead diesel engines is that under the temperature conditions at the top of the liners of such engines, cylinder liner and piston ring wear can still occur, and indeed it can be enhanced even though lubricant film breakdown does not occur.

According to the present invention there is provided a lubricant composition for lubricating a crosshead diesel engine, the composition comprising a major amount of a base oil and minor amounts of an anti-wear additive and of an extreme pressure additive, the anti-wear additive being a compound of formula X=P(OR)₃, (where X represents an oxygen or a sulfur atom, and each R, which can be the same or different, represents a phenyl, tolyl or xylyl group, or a halogenated derivative of such a group) and the extreme pressure additive being a sulfurised olefin containing from 25 to 55 percent by weight of sulfur, the weight ratio of anti-wear additive to extreme pressure additive being from 0.2:1 to 10:1, and the total base number being at least 40 (as measured by ASTM D2896 in mg of KOH/g of composition).

The invention further provides a method of lubricating a crosshead diesel engine, the method comprising lubricating the engine with a composition in accordance with the invention.

Compositions in accordance with the present invention have enabled good lubrication to be achieved between metal surfaces at elevated temperatures and high contact pressures when compared with lubricant compositions consisting of a bas oil containing either the anti-wear additive or the extreme pressure additive alone.

Particularly good and unexpected lubricant properties at elevated temperatures and pressures can be achieved in crosshead diesel engines using compositions in accordance with the present invention. Examples of particular anti-wear additives which can be used with advantage in accordance with the invention are the phosphorothionic acid esters described in British Patent Specification 1018307, and the analogous phosphoric acid esters having an oxygen atom in place of the sulfur atom of these esters. Specific anti-wear additives which can be used include tritolylphosphate, trixylylphosphate or triphenylphosphorothionate.

The sulfurised olefins used as extreme pressure additives in accordance with the invention contain from 25 to 55 percent by weight of sulfur. Particularly preferred extreme pressure additives contain from 35 to 45% by weight of sulfur. The olefinic portion of the sulfurised olefins can be derived from one or more olefin, and the olefins can be straight or branched chain, or cyclic. Furthermore, the unsaturation can be terminal or internal. Preferably, the olefins contain up to eight carbon atoms. Particularly preferred extreme pressure additives are derived from olefins containing from 3 to 6 carbon atoms. Especially preferred sulfurised olefins which can be used as extreme pressure additives in lubricant compositions of the invention are described in British Patent Specification 1308894 and U.S. Patent Specification 4204969.

The amount of extreme pressure additive should be sufficient to provide an extreme pressure effect. This will usually be provided by the presence of up to 5.0 percent of the additive based on the total weight of the composition. In general, at least 0.05 percent of an extreme pressure additive will need to be present, and compositions of the invention preferably contain from 0.05 to 0.2, more preferably from 0.1 to 1.5, and advantageously from 0.3 to 1.0 percent by weight of an extreme pressure additive based on the total weight of the composition.

The amount of anti-wear additive present is based on the amount of extreme pressure additive present. The weight ratio of anti-wear additive to extreme pressure additive should be from 0.2:1 to 10:1, preferably from 0.2:1 to 5:1, and advantageously about 0.5:1. The relative amounts of these additives is preferably adjusted to provide the compositions with good anti-wear properties under high pressures but without excessive corrosion at elevated temperatures. The amounts of anti-wear and extreme pressure additives present in order to achieve this will often be less than would be expected to provide the compositions with satisfactory low wear at high temperatures based on the known properties of the anti-wear and extreme pressure additives used.

The base oil, which can consist of a mixture of two or more oils, is preferably a hydrocarbon oil, and it can include one or more paraffinic or synthetic oils. In general, it is preferred to use a mixture of oils.

The viscosity index of the base oil should in general be at least 50, and preferably at least 70, although it will not usually be more than 180, and preferably not more than 130. The base oil preferably has a viscosity index of from 95 to 105.

Compositions used in accordance with the present invention will usually contain other additives, for example overbased additives, e.g. naphthenates, sulfonates, phenates, salicylates or carboxylates. The total base number (TBN) of the compositions should be at least 40, and preferably from 70 to 100 (as measured by ASTM D2896 in mg of KOH/g of composition). The TBN of the compositions is preferably not more than 150.

The viscosity of the compositions is preferably at least 10, and more preferably at least 15 cSt at 100°C. However, the viscosity of the base oil will usually be not more than 35, and preferably not more than 30 cSt at 100°C. Advantageously the viscosity of the oil will be from 17 to 25 cSt at 100°C.

The lubricant compositions can be prepared by known methods. Thus it is generally convenient first to heat the base oil, usually to a temperature of about 60°C, then to add any overbased additives with stirring, and finally to add the extreme pressure and anti-wear additives, again with stirring, preferably after allowing the mixture to cool.

As will be appreciated, the compositions can contain various additives used in the lubricant art, for example dispersants, antioxidants and corrosion inhibitors.

The following Examples are given by way of illustration only. All parts represent percentages by weight of the final lubricant compositions, unless stated otherwise.

### Example 1

58.96 parts of 500 SN mineral oil (viscosity index 95) and 13.0 parts of mineral oil brightstock (viscosity index 95) were blended and heated to about 60°C. 12.65 parts of overbased 250 TBN calcium phenate, 12.65 parts of overbased 300 TBN calcium sulfonate and 2.0 parts of polyalkylene succinimide were added to the blend with vigourous stirring. The resultant homogeneous mixture was cooled to about 50°C, and 0.50 part of sulfurised olefin (containing about 38% of sulfur) and 0.24 part of tritolyl phosphate (TTP) were added with stirring.

The lubricant composition produced (TBN 70.6, viscosity index 97, and viscosity 17.2 cSt at 100°C) was then tested on a standard IP 239/85 test "Extreme Pressure Properties : Friction and Wear Tests for Lubricants : Four-Ball Machine" modified to operate from ambient to 200°C, the latter temperature being approximately that at the top of the cylinder liner of a slow speed crosshead diesel engine. The results obtained are shown in the accompanying Table, weld point and initial seizure values being in kg, and scar values in mm.

### Example 2

In a similar manner to that described in Example 1, 59.04 parts of 500 SN mineral oil (viscosity index 95) and 13.0 parts of mineral oil brightstock (viscosity index 95) were blended and heated to about 60°C. 12.65 parts of overbased 250 TBN calcium phenate, 12.65 parts of overbased 300 TBN calcium sulfonate and 2.0 parts of polyalkylene succinimide were added to the blend with vigourous stirring. The resultant homogeneous mixture was cooled to about 50°C and 0.45 part of the sulfurised olefin and 0.21 part of triphenylphosphorothionate were added with stirring.

The lubricant composition produced (TBN 70.3, viscosity index 98, and viscosity 17.1 cSt at 100°C) was then tested as in Example 1, the results being shown in the accompanying Table.

### Example 3

A composition similar to that produced in Example 1 was prepared using 0.55 parts of tritolyl phosphate and 0.5 part of the sulfurised olefin, the amount of mineral oil being adjusted accordingly.

The composition was tested as in Example 1, and the results are shown in the accompanying Table.

### Example 4

A composition similar to that of Example 1 was prepared using 0.25 part of trixylyl phosphate in place of the tritolyl phosphate, the amount of mineral oil being adjusted accordingly. The composition was tested as in Example 1, and the results are given in the accompanying Table.

### Examples 5 and 6

Two lubricant compositions were prepared using the method of Example 1 but with the amounts and types of extreme pressure and anti-wear additives shown in the accompanying Table, the amount of mineral oil being adjusted accordingly. The results of the tests carried out as described in Example 1 are also given in the Table.

### Note

In the Table, the following apply:-
- Sulfide A: - Sulfurised olefin containing about 38% of sulfur
- Sulfide B: - Organic sulfide containing about 42% of sulfur
- TTP: - Tritolylphosphate
- TPPT: - Triphenylphosphorothionate
- TXP: - Trixylylphosphate

**TABLE**

| Example | Extreme pressure/anti-wear additive | Weld point | Initial Load | seizure Scar | 1 hour wear at 200°C (scar) |
|---|---|---|---|---|---|
| 1 | 0.05 Sulfide A | 340 | 165 | 1.381 | 1.010 |
| | 0.24 TTP | | | | |
| 2 | 0.45 Sulfide A | 370 | 160 | 0.756 | 0.985 |
| | 0.21 TPPT | | | | |
| 3 | 0.5 Sulfide A | 370 | 170 | 1.641 | 1.085 |
| | 0.55 TTP | | | | |
| 4 | 0.5 Sulfide A | 350 | 145 | 1.055 | 1.100 |
| | 0.24 TXP | | | | |
| 5 | 1.12 Sulfide A | 460 | 155 | 0.691 | 1.363 |
| | 0.53 TTP | | | | |
| 6 | 1.57 Sulfide B | 630 | 180 | 0.613 | 1.240 |
| | 1.0 TTP | | | | |

## Claims

1. A lubricant composition for lubricating a crosshead diesel engine, the composition comprising a major amount of a base oil and minor amounts of an anti-wear additive and of an extreme pressure additive, the anti-wear additive being a compound of formula X=P(OR)₃, (where X represents an oxygen or a sulfur atom, and each R, which can be the same or different, represents a phenyl, tolyl or xylyl group, or a halogenated derivative of such a group) and the extreme pressure additive being a sulfurised olefin containing from 25 to 55 percent by weight of sulfur, the weight ratio of anti-wear additive to extreme pressure additive being from 0.2:1 to 10:1, and the total base number being at least 40 (as measured by ASTM D2896 in mg of KOH/g of composition).

2. A composition according to claim 1, wherein each R represents a 4-tolyl or 3,5-xylyl group, or a halogenated derivative of such a group.

3. A composition according to claim 1 or claim 2, wherein each R has the same meaning.

4. A composition according to any of the preceding claims, wherein the anti-wear additive is tritolylphosphate, trixylylphosphate or triphenylphosphorothionate.

5. A composition according to any of the preceding claims, containing up to 5.0 percent of a sulfurised olefin.

6. A composition according to claim 5, containing from 0.05 to 2.0 percent of a sulfurised olefin.

7. A composition according to any of the preceding claims, having a viscosity of from 10 to 35 cSt at 100°C.

8. A composition according to any of the preceding claims, wherein the viscosity index of the base oil is from 50 to 130.

9. A composition according to any of the preceding claims, containing an overbased additive.

10. A composition according to any of the preceding claims, having a total base number (as measured by ASTM D2896 in mg of KOH/g of composition) of from 40 to 150.

11. A method of lubricating a crosshead diesel engine, the method comprising lubricating the engine with a composition according to any of the preceding claims.

## Patentansprüche

1. Schmiermittelzusammensetzung zum Schmieren einer Kreuzkopfdieselmaschine, wobei die Zusammensetzung eine größere Menge eines Basisöls und kleinere Mengen eines Antiverschleißadditivs und eines Extremdruckadditivs umfaßt, wobei das Antiverschleißadditiv eine Verbindung der Formel X=P(OR)₃ ist, (worin X ein Sauerstoff- oder Schwefelatom bedeutet und jedes R, das gleich oder verschieden sein kann, eine Phenyl-, Tolyl- oder Xylylgruppe oder ein halogeniertes Derivat einer derartigen Gruppe bedeutet) und das Extremdruckadditiv ein sulfuriertes Olefin ist, welches von 25 bis 55 Gewichtsprozent Schwefel enthält, wobei das Gewichtsverhältnis von Antiverschleißadditiv zu Extremdruckadditiv von 0,2:1 bis 10:1 ist und die Gesamtbasenzahl mindestens 40 ist (gemessen durch ASTM D2896 in mg KOH/g der Zusammensetzung).

2. Zusammensetzung nach Anspruch 1, worin jedes R eine 4-Tolyl- oder 3,5-Xylylgruppe oder ein halogeniertes Derivat einer derartigen Gruppe bedeutet.

3. Zusammensetzung nach Anspruch 1 oder Anspruch 2, worin jedes R die gleiche Bedeutung hat.

4. Zusammensetzung nach einem der vorhergehenden Ansprüche, worin das Antiverschleißadditiv Tritolylphosphat, Trixylylphosphat oder Triphenylphosphorthionat ist.

5. Zusammensetzung nach einem der vorhergehenden Ansprüche, welche bis zu 5,0 Prozent eines sulfurierten Olefins enthält.

6. Zusammensetzung nach Anspruch 5, welche von 0,05 bis 2,0 Prozent eines sulfurierten Olefins enthält.

7. Zusammensetzung nach einem der vorhergehenden Ansprüche, mit einer Viskosität von 10 bis 35 cSt bei 100°C.

8. Zusammensetzung nach einem der vorhergehenden Ansprüche, worin der Viskositätsindex des Basisöls von 50 bis 130 ist.

9. Zusammensetzung nach einem der vorhergehenden Ansprüche, welche ein überalkalisiertes Additiv enthält.

10. Zusammensetzung nach einem der vorhergehenden Ansprüche mit einer Gesamtbasenzahl (gemessen durch ASTM D2896 in mg KOH/g Zusammensetzung) von 40 bis 150.

11. Verfahren zum Schmieren einer Kreuzkopfdieselmaschine, wobei das Verfahren das Schmieren der Maschine mit einer Zusammensetzung nach einem der vorhergehenden Ansprüche umfaßt.

## Revendications

1. Composition de lubrifiant destinée à lubrifier un moteur Diesel à crosse, la composition comprenant une quantité principale d'une huile de base et des quantités mineures d'un additif anti-usure et d'un additif pression extrême, l'additif anti-usure étant un composé de la formule X=P(OR)₃, (dans laquelle X représente un atome oxygène ou un atome soufre, et chaque R, qui peut être identique ou différent, représente un groupe phényle, tolyle ou xylyle, ou un dérivé halogéné de ce groupe) et l'additif de pression extrême étant une oléfine sulfurisée contenant de 25 à 55 % en poids de soufre, le rapport en poids entre l'additif anti-usure et l'additif pression extrême étant de 0,2:1 à 10:1, et le nombre de base total étant au moins de 40 (mesuré selon ASTM D2896 en mg de KOH/g de composition).

2. Composition selon la revendication 1, dans laquelle chaque R représente un groupe 4-tolyle ou 3,5-xylyle, ou un dérivé halogéné de ce groupe.

3. Composition selon la revendication 1 ou 2, dans laquelle chaque R a la même signification.

4. Composition selon l'une quelconque des revendications précédentes, dans laquelle l'additif anti-usure est le tritolylphosphate, le trixylylphosphate ou le triphénylphosphorothionate.

5. Composition selon l'une quelconque des revendications précédentes, contenant jusqu'à 5,0 % d'un oléfine sulfurisée.

6. Composition selon la revendication 5, contenant de 0,05 à 2,0 % d'oléfine sulfurisée.

7. Composition selon l'une quelconque des revendications précédentes, ayant une viscosité allant de 10 à 35 cSt à 100°C.

8. Composition selon l'une quelconque des revendications précédentes, dans laquelle l'indice de viscosité de l'huile de base est de 50 à 130.

9. Composition selon l'une quelconque des revendications précédentes, contenant un additif surbasé.

10. Composition selon l'une quelconque des revendications précédentes, ayant un nombre de base total (mesuré selon ASTM D2896 en mg de KOH/g de composition) allant de 40 à 150.

11. Procédé de lubrification d'un moteur Diesel à crosse, le procédé comprenant la lubrification du moteur avec une composition selon l'une quelconque des revendications précédentes.
